

May 7, 1940.

H. G. SCHNETZLER

2,199,759

MANUFACTURE OF COKE

Filed June 16, 1937



INVENTOR

HARRY G. SCHNETZLER

BY *Peter H. Sullivan*

ATTORNEY

## UNITED STATES PATENT OFFICE

2,199,759

## MANUFACTURE OF COKE

Harry G. Schnetzler, Neodesha, Kans., assignor  
to Standard Oil Company, Chicago, Ill., a cor-  
poration of Indiana

Application June 16, 1937, Serial No. 148,441

8 Claims. (Cl. 202—31)

This invention relates to the coking of hydrocarbon oils and contemplates a process in which hydrocarbon oil is subjected to a prolonged digestion to thereby greatly increase the yield of 5 lump coke. In accordance with the invention, hydrocarbon oil is subjected to a coking temperature to effect conversion into a coke residue and the coke residue is digested under its contained heat.

10 My invention is concerned with a process in which the oil to be coked is heated in a heating coil or zone of restricted cross sectional area and discharged into an enlarged chamber in which the oil is maintained at a coking temperature to effect coking. I have discovered that if the material in the coking chamber be digested for a prolonged time beyond the period when any substantial quantity of distillate is formed the yield of 15 lump coke is thereby greatly increased. In ordinary coking practice it has been the custom to cool down the coked mass as rapidly as possible as soon as the flow of distillate has ceased in order to remove the coke. In accordance with my invention, the yield of lump coke may be 20 materially increased, and the hardness of the coke product increased, by maintaining the coke at an elevated temperature for a considerable period beyond that at which the flow of distillate has substantially stopped.

25 In accordance with the invention a petroleum oil such as reduced crude is passed through a heating coil wherein the oil is raised to a temperature adequate to support a coking reaction upon being discharged into an enlarged coking chamber. The heat imparted to the mass in the coking chamber by the entering stream of hot oil operates to effect the coking of the mass in the coking chamber. The vapors and gases evolved are withdrawn from the coking chamber while the liquid constituents are retained and converted into a solid coke residue. A continuous 30 stream of hot oil from the heating coil is passed into the coking chamber until the desired quantity of liquid has been introduced whereupon the introduction of heated oil is discontinued.

35 The evolution of condensable vapors continues for a time after the introduction of heated oil has ceased. If the mass in the coking chamber is permitted to remain, at an elevated temperature, a reaction will continue for a considerable 40 time, the presence of the reaction being indicated by the evolution of a relatively small quantity of fixed gas.

In order to more fully disclose the invention, 45 reference will now be had to the accompanying drawing, which is a diagrammatic sectional elevation of an apparatus adapted for the practice of the invention.

In the drawing, 10 represents a furnace in 50 which is mounted a heating coil 11 to which the

5 charging stock is introduced by pump 12. A convenient number of coking drums as 13a, 13b and 13c are shown. The heated oil is transferred from the heating coil 11 through a transfer line 14 having a ring manifold 15 through which the heated oil may be constantly circulated and diverted to the desired coking drum through one of the branch lines 15a, 15b, and 15c. The drums are provided with bottom manways 16a, 16b and 16c for the removal of the coke. The drums may 10 be conveniently equipped with coke-removal apparatus (not shown) which may consist of cables supported on wires stretched across the interior of the drum on hooks welded to the sides of the drums. The drums should be heavily insulated 15 against heat loss. The drums are equipped with vapor lines 17a, 17b and 17c respectively, manifolded to a common vapor line 18 extending to a fractionating tower 19. A branch vapor line 20 is provided, having branches 20a, 20b and 20c to 20 the respective coking drums, to provide for the passage of hot vapors from a coking drum in operation to another drum for the purpose of preheating the latter preparatory to the introduction of the heated oil from the heating coil 25 thereinto. A vapor line 21 extends to a condenser coil 22. A condensate line 23 is provided for withdrawing reflux condensate from the fractionating tower. The coking drums are equipped with blow-down lines 24a, 24b, and 24c manifolded to a gas line 25 extending to a blow-down tank 26.

The invention is particularly adapted for the treatment of heavy petroleum stocks, such as reduced crude, to effect a reduction of the heavy 35 stock to coke and produce, in addition to gasoline, a relatively large yield of condensate of the nature of gas oil suitable for charging stock to a cracking operation for conversion into gasoline. In practicing the invention with this end in view, the reduced crude is charged by the pump 12 to the heating coil 11 wherein it is heated to a temperature of about 870° F.—940° F., and discharged thence into a coking drum for conversion 40 into coke. During the time that the heated oil from the coil is being discharged into a given coking drum and for a comparatively short time after the hot oil stream has been diverted to another coke drum, the operation is accompanied 45 with the production of distillate, the evolved vapors being subjected to fractionation in the tower 19, the overhead vapors therefrom being condensed in coil 22 and the reflux condensate, which is suitable for charging stock to a cracking operation, being withdrawn from the tower 19 through the line 23. In a relatively short time 50 after the stream of hot oil from the heating coil has been diverted from a given coking drum, and as soon as the flow of distillate has substantially ceased, the valve in the vapor line of such drum, as in line 17a, 17b, or 17c, is closed and the valve 55 60

in the gas line of such drum, as in line 24a, 24b, or 24c, is opened to permit the flow of gas to the blow-down tank 26.

The mass in the coking drum is permitted to digest with retained heat for a period of time approximating at least 18 hours and preferably about 24 hours or even longer. At the beginning of the digestion period the temperature in the coking drum will be about 800° F.-850° F. The heat is largely retained during the digestion. At the end of the digestion the inner portions of the coke mass may be at temperatures approximating 800° F., and although portions near the outer surface may have dropped to about 500° F.-600° F. the average temperature may be in excess of 700° F.

The coking operation is advantageously carried on under atmospheric pressure or moderate superatmospheric pressures, such as 15-30 pounds, although the use of higher pressures is not precluded in the practice of the invention. During the digestion period there is, as stated, a relatively small evolution of gas which flows through the line 25 to the blow-down tank 26. In the early part of the digestion period the evolved gas may contain a very small proportion of waxy condensables. Upon washing the gas with water in the blowdown tower 26 a small quantity of wax slop is separated from the gas. The amount of condensables thus formed will be less than one percent of the charge to the coking drum. During the greater portion of the digestion period only a light gas is evolved.

During the digestion period it is advisable for safety purposes to introduce a very small quantity of steam into the coking drum from which the heated oil stream has been diverted in order to prevent the possibility of air getting into the coking drum from the blow-down tank. Thus, for example, assuming that drum 13a has been charged with hot oil from the heating coil to the extent desired and that the hot oil stream has been diverted to one or the other coking drums, a very small quantity of steam may be admitted into the branch transfer line 15a. This procedure will serve to insure that air does not enter the coking drum 13a from the blow-down tower 26. The quantity of steam introduced, however, should be insufficient to produce any material amount of cooling of the coke mass in the coking drum. After the coke in the coking drum has been thus digested for the required length of time the coke mass may be steamed with a relatively large quantity of steam and washed with water. The coke is then pulled from the bottom manway.

If desired, a portion or all of the reflux condensate withdrawn through line 23 may be cycled to the heating coil 11, or lighter and heavier cuts of reflux condensate may be made in the fractionating tower, with the heavy cut being cycled to the cracking coil 11 and the lighter cuts subjected to cracking in another unit. The cycling of condensate to the heating coil will normally effect an increase in the gasoline yield due primarily to the cracking of the cycle condensate in the cracking coil. It is advantageous, however, to operate without recycling condensate, or at least to only cycle a heavy cut of condensate, so that the large yield of gas oil stock, and particularly the lighter gas oil constituents, produced in the process may be subjected to cracking in a separate cracking unit under conditions better suited for the production of a gasoline of higher anti-knock quality.

In a typical operation in accordance with the invention using coking drums having a diameter of about 16 feet and a length of about 30 feet, reduced crude petroleum is charged through the heating coil 11 and thence to one of the coking drums, as 13a, for a period of about 36 hours. The reduced crude is delivered to the coking drum at a temperature approximating 900° F. The evolved vapors pass through branch line 17a and vapor line 18 to the fractionating tower 19, the overhead vapors from which are condensed in condenser coil 22 and the heavier reflux condensate from which is withdrawn through line 23. During the latter portion of the 36 hour period, for example for about 7-12 hours, the vapors from the drum 13a may be diverted into another drum, as through branch line 17b into drum 13b, thence through branch line 20b and line 20 to the fractionating tower, the withdrawal of distillate and reflux condensate being continued. In this way drum 13b may be preheated ready to receive the stream of hot oil from the heating coil 11, when the stream is diverted from the drum 13a. At the end of the 36 hour period the oil stream from the heating coil is diverted from the drum 13a into drum 13b, the flow of vapors from drum 13a being then restored to the direct passage to the fractionating tower through lines 17a and 18. In about an hour after the discontinuance of charging into drum 13a, the production of distillate from this drum will have practically ceased, at which time the vapor line 17a is closed and the gas line 24a is opened to permit the passage of gas through line 25 into the blow-down tank 26. This operation is continued for some 23 hours or until about 24 hours from the time when the heated oil stream was diverted from drum 13a, thus permitting the desired reactions to occur in the coke mass in the drum 13a. At the end of the 24 hour period steam at the rate of about 12,000 to 15,000 pounds per hour is introduced into the coking drum 13a for a period of about 15 minutes, after which water at the rate of about 100 gallons per minute is introduced for another 15 minute period. The coke is then ready to be pulled through the bottom manway 16a.

In comparing the yield of lump coke produced by the practice of my invention with the yield produced in prior methods in which heavy oil was passed through a heating coil and delivered into an insulated coking drum for coking, the yield of lump coke is taken as the proportion, of total coke produced, obtainable over a 3 inch grizzly. In the prior practice the usual amount of lump coke, as thus determined, was about 15 percent and only occasionally was it possible to obtain as high a yield as 25 percent. In practicing my invention, the yield of lump coke is very materially increased, the following examples being representative of the yields of coke produced by the practice of the invention:

| Charging stock                                       | Heating coil outlet temp. | Period of digestion | Yield of lump coke | 65 |
|------------------------------------------------------|---------------------------|---------------------|--------------------|----|
| Reduced Mid-Continent crude                          | ° F.                      | Hours               | Percent            |    |
| Mixture of crude residuum—89% Pressure tar—11% } 915 | 925                       | 28                  | 39.2               | 70 |
| Reduced Mid-Continent crude (air added)              |                           | 24                  | 57.0               |    |
|                                                      |                           | 24                  | 41.3               |    |

In the last example given in the table the reduced crude was charged to the heating coil at a 75

rate of 90 to 100 barrels per hour, and delivered into the transfer line at a temperature of 910° F. while air at the rate of 250-300 cubic feet per minute was admitted into the transfer line operating to raise the temperature about 20° F.

5 While I have described a particular embodiment of my invention for the purpose of illustration, it should be understood that various modifications and adaptations thereof which will 10 be obvious to one skilled in the art, may be made within the spirit of the invention as set forth in the appended claims.

I claim:

1. The method of coking hydrocarbon oils 15 that comprises maintaining a mass of hydrocarbons at a coking temperature with resultant evolution of condensable vapors in an enlarged coking chamber insulated against heat loss, heating a confined stream of hydrocarbon oil in an 20 elongated passageway of restricted cross sectional area to a cracking temperature and delivering into the enlarged coking chamber the resultant heated stream of hydrocarbon oil at a temperature sufficient to maintain the mass in the coking 25 chamber at a coking temperature, discontinuing the delivery of said heated stream of hydrocarbon oil to the coking chamber while retaining the residual constituents therein under their contained heat with the continued evolution of condensable vapors, and maintaining the resultant 30 coke residue therein at an elevated temperature solely under its contained heat for an extended period of time after the flow of condensable vapors has substantially ceased to thereby effect reaction 35 in the coke mass increasing the yield of lump coke, as measured by the lump coke obtainable over a three-inch grizzly.

2. The method of coking hydrocarbon oil that 40 comprises maintaining a mass of hydrocarbons in a coking zone at a coking temperature with resultant evolution of condensable vapors and conversion into a coke residue and continuing the maintenance of a coking temperature in the coking zone until such time as the evolution of condensable vapors from the coking zone has substantially 45 ceased, and then digesting the entire mass of resultant coke residue under its contained heat, without the application of either substantial cooling or heating thereto, for an extended period of time beyond that at which such evolution of condensable vapors from the coking zone has substantially ceased to thereby effect such reaction in the coke mass that upwards of approximately 40% of the total coke product, 50 upon removal from the coking zone, will consist of lump coke of the sizes obtainable over a three-inch grizzly.

3. The method of coking hydrocarbon oil that 55 comprises maintaining a mass of hydrocarbons in a coking zone at a coking temperature with resultant evolution of condensable vapors and conversion into a coke residue and continuing the maintenance of a coking temperature in the coking zone until such time as the evolution of condensable vapors from the coking zone has substantially 60 ceased, then digesting the entire mass of resultant coke residue under its contained heat, without the application of either substantial cooling or heating thereto, for a period of upwards of 18 hours beyond that at which such evolution of condensable vapors has substantially ceased to thereby effect reaction in the coke mass materially increasing the yield of lump coke, as measured by the lump coke obtainable over a 65 three-inch grizzly.

4. The method of coking hydrocarbon oil that 70 comprises maintaining a mass of hydrocarbons in a coking zone at a coking temperature with resultant evolution of condensable vapors and conversion into a coke residue and continuing the maintenance of a coking temperature in the coking zone until such time as the evolution of condensable vapors from the coking zone has substantially ceased, then digesting the entire mass of resultant coke residue while largely retaining its contained heat and maintaining the bulk of the coke mass at temperatures of the order of 700° F.-800° F. for an extended period of time beyond that at which such evolution of condensable vapors has substantially ceased to thereby effect reaction in the coke mass materially increasing the yield of lump coke, as measured by the lump coke obtainable over a three-inch grizzly.

5. The method of coking hydrocarbon oil that 75 comprises maintaining a mass of hydrocarbons in a coking zone at a coking temperature with resultant evolution of condensable vapors, delivering into the coking zone a continuous stream of hydrocarbons heated sufficiently to maintain the mass therein at a coking temperature, discontinuing the delivery of the stream of heated hydrocarbons into the coking zone, maintaining the mass in the coking zone at a coking temperature under its contained heat after discontinuing the delivery of the stream of heated hydrocarbons thereto until such time as the evolution of condensable vapors has substantially ceased, then digesting the entire mass of resultant coke residue under its contained heat, without the application of either substantial cooling or heating thereto, 80 for an extended period of time beyond that at which such evolution of condensable vapors has substantially ceased to thereby effect reaction in the coke mass materially increasing the yield of lump coke, as measured by the lump coke obtainable over a three-inch grizzly.

6. The method of coking hydrocarbon oil that 85 comprises maintaining a mass of hydrocarbons in a coking zone at a coking temperature with resultant evolution of condensable vapors, delivering into the coking zone a continuous stream of hydrocarbons heated sufficiently to maintain the mass therein at a coking temperature, discontinuing the delivery of the stream of heated hydrocarbons into the coking zone, maintaining the mass in the coking zone at a coking temperature under its contained heat after discontinuing the delivery of the stream of heated hydrocarbons thereto until such time as the evolution of condensable vapors has substantially ceased, then digesting the entire mass of resultant coke residue under its contained heat, without the application of either substantial cooling or heating thereto, for an extended period of time beyond that at which such evolution of condensable vapors has substantially ceased to thereby effect such reaction in the coke mass that upwards of approximately 40% of the total coke product, upon removal from the coking zone, will consist of lump coke of the sizes obtainable over a three-inch 90 grizzly.

7. The method of coking hydrocarbon oil that 95 comprises maintaining a mass of hydrocarbons in a coking zone at a coking temperature with resultant evolution of condensable vapors, delivering into the coking zone a continuous stream of hydrocarbons heated sufficiently to maintain the mass therein at a coking temperature, discontinuing the delivery of the stream of heated hydrocarbons into the coking zone, maintaining the

mass in the coking zone at a coking temperature under its contained heat after discontinuing the delivery of the stream of heated hydrocarbons thereto until such time as the evolution of condensable vapors has substantially ceased, then digesting the entire mass of resultant coke residue while largely retaining its contained heat and maintaining the bulk of the coke mass at temperatures approximating 700° F.-800° F. for an extended period of time beyond that at which such evolution of condensable vapors has substantially ceased to thereby effect reaction in the coke mass materially increasing the yield of lump coke, as measured by the lump coke obtainable over a three-inch grizzly.

8. The method of coking hydrocarbon oil that comprises heating a confined stream of hydrocarbon oil in an elongated passageway of restricted cross-sectional area to a temperature within the range of 870° F.-940° F., continuously passing the heated stream of hydrocarbon oil into

an enlarged coking chamber insulated against heat loss to maintain a mass of hydrocarbons therein at a coking temperature with resultant evolution of condensable vapors, discontinuing the delivery of the heated stream of hydrocarbon oil into the coking chamber while continuing the maintenance of the mass therein at a coking temperature until such time as the evolution of condensable vapors has substantially ceased, then digesting the entire mass of resultant coke residue in the coking chamber while largely retaining its contained heat and maintaining the bulk of the coke mass therein at temperatures of the order of 700° F.-800° F. for an extended period of time beyond that at which such evolution of condensable vapors from the coking chamber has substantially ceased to thereby effect reaction in the coke mass materially increasing the yield of lump coke, as measured by the lump coke obtainable over a three-inch grizzly.

HARRY G. SCHNETZLER.

20